# EUROPEAN PATENT APPLICATION

(11) **EP 1 637 580 A1**
(43) Date of publication of application: **22.03.2006**
(21) Application number: 05017288.1
(22) Date of filing: 09.08.2005
(51) Int. Cl.: C10M 171/04, C10M 171/02, C08L 23/00, C08L 25/00, C10N 20/04, C10N 20/02, C10N 40/04, C10N 40/25, C10N 70/00

(54) **Viscosity index modifying additives for lubricating compositions**

(30) Priority: 17.09.2004 US 943375
(71) Applicant: Afton Chemical Corporation, Richmond, VA 23219 (US)
(72) Inventor: Srinivasan, Sanjay, Midlothian Virginia 23113 (US); Song, Yoon Soo, Richmond Virginia 23233 (US); Strukl, Joseph Stephen, Midlothian Virginia 23112 (US); Growcott, Peter, Hartley Wintney Hampshire RG27 8TE (GB); Griffin, Paul G., Glen Allen Virginia 23059 (US); Duggal, Akhilesh, Midlothian Virginia 23112 (US)
(74) Representative: Schwabe - Sandmair - Marx

(57) **Abstract**

A lubricant composition method of using the lubricant composition. The lubricant composition contains a base oil of lubricating viscosity and from about 5 to about 30 percent by weight of an additive comprising a shear stable olefin copolymer derived from a copolymer having a number average molecular weight ranging from about 50,000 to about 250,000. The shear stable olefin copolymer has a shear stability index of less than about 40, a polydispersity of not more than about 1.5, and a thickening efficiency of greater than about 1.8, and provides viscosity index improving properties to the lubricant composition.

## Description

### TECHNICAL FIELD

The following disclosure is directed to lubricants, lubricant compositions and additives, lubricated parts and engines, and methods for lubricating moving parts.

### BACKGROUND

Lubricating oils used in gasoline and diesel crankcases include a natural and/or synthetic basestock and one or more additives to impart desired characteristics to the lubricant. Such additives typically include ashless dispersant, metal detergent, antioxidant and antiwear components, which may be combined in a package, sometimes referred to as a detergent inhibitor (or D1) package.

Multigrade oils usually also contain one or more viscosity modifiers which are relatively long chain polymers. Such polymers may be functionalized to provide other properties when they are known as multifunctional viscosity modifiers, but primarily act to improve the viscosity characteristics of the oil over a desired operating temperature range. The viscosity modifier acts to increase viscosity at high temperature to provide more protection to the engine at high speeds, without unduly increasing viscosity at low temperatures which would otherwise make starting a cold engine difficult. High temperature performance is usually measured in terms of the kinematic viscosity (kV) at 100° C. (ASTM D445), while low temperature performance is measured in terms of cold cranking simulator (CCS) viscosity (ASTM D5293, which is a revision of ASTM D2602) ), mini-rotary viscometer (MRV; ASTM D4684), or scanning brookfield or gel index (ASTM D5133)..

Viscosity grades are defined by the SAE Classification system (SAE J300) according to the foregoing temperature measurements. Multigrade oils meet the requirements of both low temperature and high temperature performance and are thus referenced to both the relevant grades.

Shear stability is a measure of the ability of an oil to resist permanent viscosity loss under high shear - the more shear stable an oil the smaller the viscosity loss when subjected to shear. Polymeric viscosity modifiers, which make a significant contribution to kV 100° C., are not entirely shear stable. Such polymeric viscosity modifiers are characterized by a shear stability index (SSI).

An oil or additive that exhibits relatively high shear stability will have an SSI that is relatively low. Typically, higher molecular weight polymers used in lubricating oil applications have poor shear stability (i.e., high SSI). However, viscosity modifiers with relatively low SSI require higher treat rates due to their relatively lower molecular weights and therefore lead to an increase in total formulation costs. Multigrade oils often have poor shear stability unless they use expensive viscosity modifiers having low SSI. Poor shear stability requires the oils to be blended to a higher initial kV 100 °C. which may result in poor fuel economy. Accordingly, there is a need for improved viscosity modifiers which are relatively shear stable and more cost effective to use in lubricant composition.

### SUMMARY OF THE EMBODIMENTS

In one embodiment herein is presented a lubricated surface. The lubricated surface includes a thin film coating of a lubricant composition containing a base oil of lubricating viscosity and from about 5 to about 30 percent by weight of an additive comprising a shear stable olefin copolymer derived from a copolymer having a number average molecular weight ranging from about 50,000 to about 250,000. The shear stable olefin copolymer has a shear stability index of less than about 40, a polydispersity of not more than about 1.5, and a thickening efficiency of greater than about 1.8.

In another embodiment, there is provided a vehicle having moving parts and containing a lubricant for lubricating the moving parts. The lubricant contains an oil of lubricating viscosity and from about 5 to about 30 percent by weight of an additive comprising a shear stable olefin copolymer derived from a copolymer having a number average molecular weight ranging from about 50,000 to about 250,000. The shear stable olefin copolymer has a shear stability index of less than about 40, a polydispersity of not more than about l .5, and a thickening efficiency of greater than about 1.8.

In yet another embodiment there is provided a method of lubricating moving parts. The method includes contacting the moving parts with a lubricant composition containing a lubricant additive. The lubricant additive includes a diluent or carrier oil and from about 5 to about 95 percent by weight of a shear stable olefin copolymer derived from a copolymer having a number average molecular weight ranging from about 50,000 to about 250,000. The shear stable olefin copolymer has a shear stability index of less than about 40, a polydispersity of not more than about 1.5, and a thickening efficiency of greater than about 1.8. The lubricant composition contains from about 5 to about 30 percent by weight of the additive based on a total weight of the lubricant composition.

A further embodiment of the disclosure provides a method for improving the viscosity index of a lubricant composition. The method includes mixing with the lubricant composition from about 5 to about 30 percent by weight of an additive comprising a shear stable olefin copolymer derived from a copolymer having a number average molecular weight ranging from about 50,000 to about 250,000. The shear stable olefin copolymer has a shear stability index of less than about 40, a polydispersity of not more than about 1.5, and a thickening efficiency of greater than about 1.8.

An advantage of the shear stable copolymer as described herein is that the polymer exhibits improved thickening efficient at a lower polymer loading. Another advantage of the shear stable copolymer is that it may be made using an amorphous lower ethylene containing copolymer, e.g., a copolymer having an ethylene content in the range of from about 40% to about 55% by weight. In addition to the shear stable olefin copolymers, the disclosure may also be applicable to shear stable star polymers based on styrene-isoprene chemistry.

### BRIEF DESCRIPTION OF THE DRAWINGS:

Further features and advantages of the embodiments will become apparent by reference to the detailed description of preferred embodiments when considered in conjunction with the following drawings, in which like reference numbers denote like elements throughout the several views, and wherein:
FIG. 1 is a shear stability index profile of a mechanically sheared olefin copolymer according to the disclosure;
FIG. 2 is a polydispersity profile for a mechanically sheared olefin copolymer according to the disclosure;
FIG. 3 is a graphical representation of a viscosity profile for a mechanically sheared olefin copolymer according to the disclosure;
FIG. 4 is a graphical representation of an olefin copolymer according to the disclosure in a process oil illustrating a change in viscosity during mechanical shearing compared to conventional olefin copolymers prepared under a high temperature extruder shearing and direct finishing process; and
FIG. 5 is a thickening efficiency profile for a mechanically sheared olefin copolymer according to the disclosure compared to a thickening efficiency of conventional olefin copolymers prepared under a high temperature extruder shearing and direct finishing process.

### DETAILED DESCRIPTION OF THE PREFERRED EMBODIMENTS

As used herein, the term "hydrocarbyl substituent" or "hydrocarbyl group" is used in its ordinary sense, which is well-known to those skilled in the art. Specifically, it refers to a group having a carbon atom directly attached to the remainder of the molecule and having a predominantly hydrocarbon character. Examples of hydrocarbyl groups include:
(1) hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form an alicyclic radical);
(2) substituted hydrocarbon substituents, that is, substituents containing non-hydrocarbon groups which, in the context of the description herein, do not alter the predominantly hydrocarbon substituent (e.g., halo (especially chloro and fluoro), hydroxy, alkoxy, mercapto, alkylmercapto, nitro, nitroso, and sulfoxy);
(3) hetero-substituents, that is, substituents which, while having a predominantly hydrocarbon character, in the context of this description, contain other than carbon in a ring or chain otherwise composed of carbon atoms. Hetero-atoms include sulfur, oxygen, nitrogen, and encompass substituents such as pyridyl, furyl, thienyl and imidazolyl. In general, no more than two, preferably no more than one, non-hydrocarbon substituent will be present for every ten carbon atoms in the hydrocarbyl group; typically, there will be no non-hydrocarbon substituents in the hydrocarbyl group.

In all of the embodiments of the disclosure, a particular lubricant component or additive is provided. The additive is referred to generally as a multi-functional viscosity index modifier. Specifically, the lubricant additive includes a shear stable olefin copolymer derived from a copolymer having a number average molecular weight ranging from about 15,000 to about 500,000 or more. The shear stable olefin copolymer may have a shear stability index of less than about 40 and a polydispersity of less than or equal to about 1.5. As described herein, shear stable olefin copolymer is dissolved in a suitable solvent such as Solvent Neutral 150 to provide the additive component.

A wide variety of copolymers and terpolymers may be used as starting materials for making the shear stable copolymer. The copolymers are referred to generally as olefin copolymers, however, the disclosed embodiments may also be applicable to copolymers derived from styrene-isoprene. The copolymers typically have number average molecular weights of from about 15,000 to about 500,000; preferably about 20,000 to about 300,000, and more preferably from about 100,000 to about 200,000. The shear stable copolymers generally have a narrow range of molecular weight, as determined by the ratio of weight-average molecular weight (Mw) to number-average molecular weight (Mn), referred to hereinafter as "polydispersity." Suitable olefin copolymers have a polydispersity of less than 10, preferably less than 7, and more preferably 4 or less. The (Mn) and (Mw/Mn) of the copolymers are measured by the well known techniques of vapor phase osmometry (VPO), membrane osmometry and gel permeation chromatography. The shear stable copolymers derived from the olefin copolymers may have a polydispersity of less than or equal to about 1.5.

In general, shear stable copolymers having a narrow range of molecular weight may be obtained by relatively low temperature mechanical shearing. Conventional copolymer shearing is conducted at temperatures above about 100° C. (212° F.) in an extrusion shearing process. By contrast, shearing of the copolymers according to the disclosure is conducted at a temperature below about 100° C. (212° F.), typically from about 35° C. (95° F.) to about 85° C. (135° F.) in a homogenizer. Accordingly, the term "relatively low temperature" means a temperature below a temperature used in a conventional extrusion shearing process for shearing copolymers.

The homogenizer used in the process may be any type capable of developing a pressure in excess of 500 pounds per square inch wherein the product is subjected to high shearing action upon release of said pressure. Typical of the homogenizers which may be used are those of the type conventionally used in the homogenization of dairy products and in the preparation of emulsions utilized as polishing compounds, cosmetics, pharmaceuticals and liquid soaps. The copolymers may be sheared using multiple passes through the homogenizer, for example from about 2 to about 10 passes through the homogenizer.

The olefin copolymer sheared in the homogenizer may be prepared from ethylene and ethylenically unsaturated hydrocarbons including cyclic, alicyclic and acyclic, compounds containing from 3 to 28 carbons, e.g. 2 to 18 carbons. The ethylene copolymers may contain from about 15 to about 90 wt. % ethylene, preferably, from about 30 to about 80 wt. % of ethylene, and most preferably less than about 70 wt. % ethylene. The copolymers may also contain from about 10 to about 85 wt. %, preferably 20 to 70 wt. % of one or more C₃ to C₂₈, preferably C₃ to C₁₈ more preferably C₃ to C₁₀, unsaturated hydrocarbons, preferably alpha olefins.

Copolymers of ethylene and propylene are most preferred. However, other alpha-olefins suitable in place of propylene to form the copolymer, or to be used in combination with ethylene and propylene, to form a terpolymer, tetrapolymer, etc., include, but are not limited to, 1-pentene, 1-hexene, 1-heptene, 1-octene, 1-nonene, 1-decene, etc.; also branched chain alpha-olefins, such as 4-methyl-1-penterie, 4-methyl-1-hexene, 5-methylpentene-1, 4,4-dimethyl-1-pentene, and 6-methylheptene-1, etc., and mixtures thereof.

The term copolymer as used herein, unless otherwise indicated, includes terpolymers, tetrapolymers, interpolymers, etc., of ethylene and C₃₋₂₈ alpha-olefin and/or a non-conjugated diolefin or mixtures of such diolefins which may also be used. Such materials may contain minor amounts of other olefinic monomers so long as the basic characteristics of the olefin copolymers are not materially changed. The amount of the non-conjugated diolefin will generally range from about 0.5 to 20 mole percent, preferably about 1 to about 7 mole percent, based on the total amount of ethylene and alpha-olefin present.

Representative examples of non-conjugated dienes that may be included in a terpolymer include straight chain acyclic dienes such as 1,4-hexadiene; 1,5-heptadiene; 1,6-octadiene; branched chain acyclic dienes such as 5-methyl-1,4-hexadiene; 3,7-dimethyl 1,6-octadiene; 3,7-dimethyl-1,7-octadiene; and the mixed isomers of dihydro-myrcene and dihydro-cymene; single ring alicyclic dienes such as 1,4-cyclohexadiene; 1,5-cyclooctadiene; 1,5-cyclododecadiene; 4-vinylcyclohexene; 1-allyl-4-isopropylidene cyclohexane; 3-allyl-cyclopentene; 4-allyl-cyclohexene and 1-isopropenyl-4-(4-butenyl) cyclohexane; multi-single ring alicyclic dienes such as 4,4-dicyclopentenyl and 4,4-dicyclohexenyl dienes; multi-ring alicyclic fused and bridged ring dienes such as tetrahydroindene; methyl tetrahydroindene; dicyclopentadiene; bicyclo (2.2.1.) hepta-2,5-diene; alkyl, alkenyl, alkylidene, cycloalkenyl and cycloalkylidene norbomenes such as: ethyl norbomene; 5-methylene-6-methyl-2-norbomene; 5-methylene-6,6-dimethyl-2-norbomene; 5-propenyl-2-norbomene; 5-(3-cyclopentenyl)2-norbomene and 5-cyclohexylidene-2-norbomene; norbomadiene; etc.

Specifically, the shear stable olefin copolymer may be derived from the polymerization of ethylene-propylene monomers, ethylene-propylene-diene monomers, styrene-neoprene monomers, styrene-isoprene monomers, and the like.

Ethylene-propylene or higher alpha-olefin copolymers may consist of from about 15 to about 80 weight percent ethylene and from about 85 to about 20 weight percent C₃ to C₂₃ alpha-olefin with the preferred weight ratios being from about 35 to about 75 weight percent ethylene and from about 65 to about 25 weight percent of a C₃ to C₂₃ alpha-olefin, with the more preferred proportions being from about 50 to less than about 70 weight percent ethylene and about 50 to about 30 weight percent C₃ to C₂₃ alpha-olefin, and the most preferred proportions being from about 55 to about 65 weight percent ethylene and from about 45 to about 35 weight percent C₃ to C₂₃ alpha-olefin.

Also included among the olefin copolymers for making the shear stable olefin copolymers as described herein are those olefin copolymers which have been functionalized by means of a free radical graft reaction or a graft polymerization reaction. Such grafted copolymers are themselves well known to those skilled in the art.

Graft monomers for functionalizing olefin copolymers are the derivatives of olefinically unsaturated carboxylic monomers such as, maleic anhydride, acrylic or methacrylic acid, or their esters, graft monomers which are likewise known to those skilled in the art. Typically, acrylic and methacrylic acid derivative contain 4 to 16 carbon atoms. Particularly preferred among the group of acrylic or methacrylic graft monomers are glycidyl methacrylate, methylacrylate, methylmethacrylate, ethylmethacrylate and aminopropylmethacrylate, and acrylamide.

Another group of graft monomers which can be used to functionalize the olefin copolymers are vinyl amines containing 2 to 25 carbon atoms, and preferably heterocyclic vinyl amines. Such amines are themselves known as functionalizing graft monomers and include allylamines, N-vinylpyridines, N-vinylpyrrolidones, vinyl lactams, vinylcarbazoles, vinylimidazoles and vinylthiazoles as represented by 2-vinylpyridine, N-vinylpyrrolidone, vinyl caprolactam, 1-vinylimidazole, allylamine, 4-methyl-5-vinylthiazole and 9-vinylcarbazole. Such graft monomers are described in detail in U.S. Pat. No. 4,340,689, the disclosure of which is incorporated herein by reference.

As it will be appreciated by those skilled in the art, other vinyl monomers described in the prior art as suitable for functionalizing olefin copolymers may likewise be used in the practice of the present invention. Examples of such further vinyl compounds are the vinyl silanes and vinyl-benzyl halides as represented by vinyltrimethoxysilane, vinyldiethychlorosilane, vinylbenzylchloride and the like. Further descriptions of suitable silane graft monomers are described in U.S. Pat. No. 4,340,689, the disclosure of which is incorporated herein by reference.

The shear stable olefin copolymer of the embodiments described herein is advantageously incorporated into lubricating compositions. The shear stable olefin copolymer may be added directly to the lubricating oil composition. In one embodiment, however, the copolymer is diluted with a substantially inert, normally liquid organic diluent such as mineral oil, synthetic oil (e.g., ester of dicarboxylic acid), naptha, alkylated (e.g., C₁₀ -C₁₃ alkyl) benzene, toluene or xylene to form an additive concentrate. The shear stable olefin copolymer concentrate usually contain from about 0% to about 99% by weight diluent oil.

In the preparation of lubricating oil formulations it is common practice to introduce the additives in the form of 1 to 99 wt. % active ingredient concentrates in hydrocarbon oil, e.g. mineral lubricating oil, or other suitable solvent. Usually these concentrates may be added with 0.05 to 10 parts by weight of lubricating oil per part by weight of the additive package in forming finished lubricants, e.g. crankcase motor oils. The purpose of concentrates, of course, is to make the handling of the various materials less difficult and awkward as well as to facilitate solution or dispersion in the final blend.

Lubricant compositions made with the shear stable olefin copolymers described above are used in a wide variety of applications. For compression ignition engines and spark ignition engines, it is preferred that the lubricant compositions meet or exceed published GF-4 or API-CI-4 standards. Lubricant compositions according to the foregoing GF-4 or API-CI-4 standards include a base oil and an oil additive package to provide a fully formulated lubricant. The base oil for lubricants according to the disclosure is an oil of lubricating viscosity selected from natural lubricating oils, synthetic lubricating oils and mixtures thereof. Such base oils include those conventionally employed as crankcase lubricating oils for spark-ignited and compression-ignited internal combustion engines, such as automobile and truck engines, marine and railroad diesel engines, and the like.

Natural oils include animal oils and vegetable oils (e.g., castor oil, lard oil), liquid petroleum oils and hydrorefined, solvent-treated or acid-treated mineral lubricating oils of the paraffinic, naphthenic and mixed paraffinic-naphthenic types. Oils of lubricating viscosity derived from coal or shale are also useful base oils. The synthetic lubricating oils used in this invention include one of any number of commonly used synthetic hydrocarbon oils, which include, but are not limited to, poly-alpha-olefins, alkylated aromatics, alkylene oxide polymers, interpolymers, copolymers and derivatives thereof here the terminal hydroxyl groups have been modified by esterification, etherification etc, esters of dicarboxylic acids and silicon-based oils.

Fully formulated lubricants conventionally contain an additive package, referred to herein as a dispersant/inhibitor package or DI package, that will supply the characteristics that are required in the formulations. Suitable DI packages are described for example in U.S. Patent Nos. 5,204,012 and 6,034,040 for example. Among the types of additives included in the additive package are detergents, dispersants, friction modifiers, seal swell agents, antioxidants, foam inhibitors, lubricity agents, rust inhibitors, corrosion inhibitors, demulsifiers, viscosity index improvers, and the like. Several of these components are well known to those skilled in the art and are preferably used in conventional amounts with the additives and compositions described herein.

For example, ashless dispersants include an oil soluble polymeric hydrocarbon backbone having functional groups that are capable of associating with particles to be dispersed. Typically, the dispersants comprise amine, alcohol, amide, or ester polar moieties attached to the polymer backbone often via a bridging group. The ashless dispersants may be, for example, selected from oil soluble salts, esters, amino-esters, amides, imides, and oxazolines of long chain hydrocarbon substituted mono and dicarboxylic acids or their anhydrides; thiocarboxylate derivatives of long chain hydrocarbons; long chain aliphatic hydrocarbons having a polyamine attached directly thereto; and Mannich condensation products formed by condensing a long chain substituted phenol with formaldehyde and a polyalkylene polyamine.

Oxidation inhibitors or antioxidants reduce the tendency of base stocks to deteriorate in service which deterioration can be evidenced by the products of oxidation such as sludge and varnish-like deposits on the metal surfaces and by viscosity growth. Such oxidation inhibitors include hindered phenols, alkaline earth metal salts of alkylphenol thioesters having preferably C₅ to C₁₂ alkyl side chains, calcium nonylphenol sulfide, ashless oil soluble phenates and sulfurized phenates, phosphosulfurized or sulfurized hydrocarbons, phosphorus esters, metal thiocarbamates and oil soluble copper compounds as described in U.S. Pat. No. 4,867,890.

Rust inhibitors selected from the group consisting of nonionic polyoxyalkylene polyols and esters thereof, polyoxyalkylene phenols, and anionic alkyl sulfonic acids may be used.

A small amount of a demulsifying component may be used. A preferred demulsifying component is described in EP 330,522. It is obtained by reacting an alkylene oxide with an adduct obtained by reacting a bis-epoxide with a polyhydric alcohol. The demulsifier should be used at a level not exceeding 0.1 mass % active ingredient. A treat rate of 0.001 to 0.05 mass % active ingredient is convenient.

Pour point depressants, otherwise known as lube oil flow improvers, lower the minimum temperature at which the fluid will flow or can be poured. Such additives are well known. Typical of those additives which improve the low temperature fluidity of the fluid are C₈ to C₁₈ dialkyl fumarate/vinyl acetate copolymers, polyalkylmethacrylates and the like.

Foam control can be provided by many compounds including an antifoamant of the polysiloxane type, for example, silicone oil or polydimethyl siloxane.

Seal swell agents, as described, for example, in U.S. Patent Nos. 3,974,081 and 4,029,587, may also be used.

Each of the foregoing additives, when used, is used at a functionally effective amount to impart the desired properties to the lubricant. Thus, for example, if an additive is a corrosion inhibitor, a functionally effective amount of this corrosion inhibitor would be an amount sufficient to impart the desired corrosion inhibition characteristics to the lubricant. Generally, the concentration of each of these additives, when used, ranges up to about 20% by weight based on the weight of the lubricating oil composition, and in one embodiment from about 0.001% to about 20% by weight, and in one embodiment about 0.01% to about 10% by weight based on the weight of the lubricating oil composition.

### Example

Four fully formulated lubricant compositions were made and the viscometric and shear strength properties of the compositions were compared. Each of the lubricant compositions contained a conventional DI package providing 11 percent by weight of the lubricant composition. The DI package contained conventional amounts of detergents, dispersants, antiwear additives, friction modifiers, antifoam agents, and antioxidants. The formulations also contained about 0.1 percent by weight pour point depressant, about 58 to 64 percent by weight 150 solvent neutral oil, about 12 to 18 percent by weight 600 solvent neutral oil. Samples 1-3 provide the characteristics of commercially available olefin copolymers as viscosity modifiers. Sample 4 provides the characteristics of a shear stable olefin copolymer made according to the disclosure.

In the tables, the following abbreviations are used:
VII - viscosity index improver
KV - kinematic viscosity
CCS - cold cranking simulator
MRV - mini rotary viscometer ― tests conducted according to ASTM D4684
HTHS - high temperature high shear - tests conducted according to ASTM D-4683, D-4781, and D-5481.

**Table 1**

| Sample # | 1 | 2 | 3 | 4 |
|---|---|---|---|---|
| Viscosity Grade | 15W50 | 15W50 | 15W50 | 15W50 |
| | | | | |

| **Components** | **Wt.%** | **Wt.%** | **Wt.%** | **Wt.%** |
|---|---|---|---|---|
| HiTEC® 9386¹ | 11.00 | 11.00 | 11.00 | 11.00 |
| HiTEC® 672 ² | 0.10 | 0.10 | 0.10 | 0.10 |
| ESSO 150 solvent neutral | 63.60 | 63.00 | 58.20 | 63.50 |
| ESSO 600 solvent neutral | 12.40 | 13.50 | 17.30 | 12.00 |

| **Viscosity Index Modifier** | | | | |
|---|---|---|---|---|
| HiTEC® 5748³ | 12.90 | 0.00 | 0.00 | 0.00 |
| LUBRIZOL 7077⁴ | 0.00 | 12.40 | 0.00 | 0.00 |
| PARATONE 8006⁵ | 0.00 | 0.00 | 13.40 | 0.00 |
| Shear Stable ethylene/propylene Copolymer (50 wt. % ethylene) | 0.00 | 0.00 | 0.00 | 13.40 |
| | | | | |
| Total | 100.00 | 100.00 | 100.00 | 100.00 |

**Table 2**

| Sample # | 1 | 2 | 3 | 4 |
|---|---|---|---|---|
| **Lubricant Properties** | | | | |
| Polymer content in VII (weight %) | 13.12 | 12.61 | 10.27 | 9.88 |
| Polymer loading in blend (grams) | 1.69 | 1.56 | 1.38 | 1.32 |
| KV at 100 °C. (cSt) | 18.98 | 19.06 | 19.02 | 18.96 |
| KV at 40° C. (cSt) | 144.80 | 146.2 | 144.4 | 146.6 |
| Viscosity index | 149 | 149 | 150 | 147 |
| CCS at -20° C. (cP) (7000 cP max.) | 6776 | 6897 | 6653 | 6840 |
| MRV TP-1@-25°C, cP | 44900 | 47300 | 0 | 40800 |
| MRV Yield Stress | <35 | <35 | <140 | <35 |
| Noack Volatility, % | 11.4 | 10.6 | 10.1 | 10.4 |
| HTHS at150°C. (cP) | 4.89 | 4.95 | 4.63 | 4.79 |
| KV at 100° C. after 30 cycle Bosch shear | 16.29 | 16.55 | 16.03 | 16.16 |
| KV at 100° C. % viscosity loss (15% max.) | 14.17 | 13.14 | 15.72 | 14.77 |
| Shear stability Index (SSI, %) | 23.60 | 20.60 | 24.20 | 24.90 |

| | | | | |
|---|---|---|---|---|
| ¹HiTEC® 9386 is a commercially available DI package available from Afton Chemical Corporation of Richmond, Virginia | | | | |
| ²HiTEC® 672 is a commercially available pour point depressant available from Afton Chemical Corporation | | | | |
| ³HiTEC® 5748 is a olefin copolymer made by an extrusion shearing process and is available from Afton Chemical Corporation | | | | |
| ⁴LUBRIZOL 7077 is an olefin copolymer having an ethylene content of about 50 weight percent and is available from Lubrizol Corporation of Wickliffe, Ohio. (The table results are from an average of two batches of LUBRIZOL 7077) | | | | |
| ⁵PARATONE 8006 is an olefin copolymer having an ethylene content of about 70 weight percent and is available from Chevron Oronite Company LLC of Houston, Texas. | | | | |

As seen in the foregoing Tables 1 and 2, sample 4 provides a highly efficient viscosity modifier. Compared with samples 1-3, sample 4 had the lowest polymer loading in the lubricant composition (1.32 versus 1.38 to 1.69 for samples 1-3). Sample 4 also had the highest shear stability index (SSI) and passed the MRV tests and CCS test, whereas, sample 3 failed the MRV test and viscosity loss test. Overall, sample 4 exhibited improved viscometric and shear strength properties over commercially available ethylene-based olefin copolymer products.

In order to make shear stable olefin copolymers according to the disclosure, 10 parts by weight ethylene/propylene copolymer having a number average molecular weight as determined by gas phase chromatography (GPC) of 179,192 and a weight average molecular weight of 332,930 was mixed with 90 parts by weight of process oil. The oil and copolymer mixture was cycled through a GAULIN homogenizer from 1 to 10 times to provide a shear stable olefin copolymer having a polydispersity of less than 1.5.

Properties of the olefin copolymer after zero to ten passes through the homogenizer are provided in the following table and FIGS. 1-3. FIGS. 4-5 provide a visual comparison of the thickening efficiency and kinematic viscosity of the olefin copolymer after zero to ten passes with the same properties of HiTEC® 5748 and LUBRIZOL 7077 (LZ 7077) (Samples 6 and 7, respectively). The comparisons were conducted with one percent olefin copolymer in a reference oil having a viscosity as indicated in the table. The kinematic viscosity at 100° C. of the samples was estimated by thermogravimetric analysis (TGA) by dissolving one weight percent of each sample in about a five centistokes reference oil (FIG. 4).

**Table 3**

| Sample No. | 1 | 2 | 3 | 4 | 5 | 6 | 7 |
|---|---|---|---|---|---|---|---|
| No. of passes through Homogenizer | 0 | 4 | 6 | 8 | 10 | ---- | ---- |
| KV at 100° C. (cSt) | 5422 | 1685 | 1299 | 1176 | 1048 | 1010 | 1212 |
| KV at 40°C. (cSt) | 78489 | 21084 | 17234 | 14878 | 13109 | 13290 | 15153 |
| VI | 385.9 | 332.8 | 321.0 | 309.3 | 303.4 | 295.4 | 313.0 |
| % Crystallinity | 2.47 | 2.32 | 2.63 | 2.79 | 2.59 | 2.30 | 2.68 |
| TGA/N2 (wt. % Polymer) | 9.635 | 9.638 | 9.668 | 9.568 | 9.627 | 12.97 | 12.80 |
| Wt. % process oil | 89.77 | 89.77 | 89.59 | 89.38 | 89.43 | 86.49 | 86.59 |
| Mn | 179192 | 163277 | 152061 | 153749 | 139436 | 72972 | 93130 |
| Mw | 332930 | 231655 | 209057 | 202834 | 183335 | 147926 | 147853 |
| Pd | 1.86. | 1.42 | 1.37 | 1.32 | 1.31 | 2.03 | 1.59 |

**Table 4**

| Sample No. | 1 | 2 | 3 | 4 | 5 | 6 | 7 |
|---|---|---|---|---|---|---|---|
| No. of passes through Homogenizer | 0 | 4 | 6 | 8 | 10 | ---- | ---- |
| KV at 100° C. in Ref. Oil (Est. by TGA) | 13.784 | 11.305 | 10.822 | 10.614 | 10.501 | 8.79 | 9.05 |
| Thickening Power (by TGA) | 8.81 | 6.33 | 5.85 | 5.64 | 5.53 | 3.82 | 4.07 |
| Thickening Efficiency (by TGA) | 2.941 | 2.369 | 2.243 | 2.187 | 2.156 | 1.717 | 1.713 |
| KV at 100° C. in Ref. oil before shearing | 11.06 | 10.92 | 10.47 | 10.31 | 10.11 | ----- | 10:86 |
| KV at 100° C. in Ref. oil after shearing | 7.99 | 9.00 | 8.95 | 8.94 | 8.91 | ------ | 9.72 |
| KV at 100° C. of Ref. Oil | 4.89 | 4.95 | 4.95 | 4.95 | 4.95 | ------ | 4.95 |
| % Viscosity Loss | 26.76 | 17.58 | 14.52 | 13.29 | 11.87 | ------ | 10.5 |
| SSI % | 49.76 | 32.16 | 27.54 | 25.56 | 23.26 | 24 | 19.29 |

As shown by the foregoing tables and FIGS. 1-5, a shear stable copolymer made by passing the copolymer through ten or more passes of a homogenizer can be tailored to provide a viscosity modifier that meets the shear stability index (SSI) requirement of about 23 (Sample 5), and has significantly higher thickening efficiency (Sample 5) compared to conventional olefin copolymer viscosity modifiers (Samples 6 and 7). Mechanical shearing of an olefin copolymer has an added benefit of providing a shear stable olefin copolymer having a polydispersity of less than 1.5 (Sample 5, Table 3).

At numerous places throughout this specification, reference has been made to a number of U.S. Patents. All such cited documents are expressly incorporated in full into this disclosure as if fully set forth herein.

The foregoing embodiments are susceptible to considerable variation in its practice. Accordingly, the embodiments are not intended to be limited to the specific exemplifications set forth hereinabove. Rather, the foregoing embodiments are within the spirit and scope of the appended claims, including the equivalents thereof available as a matter of law.

The patentees do not intend to dedicate any disclosed embodiments to the public, and to the extent any disclosed modifications or alterations may not literally fall within the scope of the claims, they are considered to be part hereof under the doctrine of equivalents.

## Claims

1. A lubricant composition comprising a base oil component of lubricating viscosity and an additive comprising a shear stable olefin copolymer derived from a copolymer having a number average molecular weight ranging from about 50,000 to about 250,000, wherein the shear stable olefin copolymer has a shear stability index of less than about 40, a polydispersity of not more than about 1.5, and a thickening efficiency of greater than about 1.8.

2. The lubricant composition of claim 1, wherein the additive is comprised in an amount of from about 5 to about 30 percent by weight based on a total amount of lubricant composition.

3. The lubricant composition of claim 1 or claim 2, wherein the shear stable copolymer is derived from the group consisting of ethylene-propylene monomers, ethylene-propylene-diene monomers, styrene-isoprene, and styrene-neoprene monomers.

4. The lubricant composition of one of the preceding claims, wherein the shear stable copolymer comprises an olefin copolymer mechanically sheared in a homogenizer.

5. The lubricant composition of one of claims 1 to 3, wherein the shear stable copolymer is derived from a relatively low temperature, homogenized copolymer.

6. The lubricant composition of one of the preceding claims, wherein each monomeric unit of the shear stable copolymer contains from about 2 to about 10 carbon atoms.

7. The lubricant composition of one of the preceding claims, wherein the shear stable copolymer comprises an amorphous ethylene containing copolymer having an ethylene content below about 70 percent by weight.

8. Use of a lubricant composition of one of claims 1 to 7 as a thin film coating on a lubricated surface.

9. The use of claim 8, wherein the lubricated surface comprises an engine drive train, an internal surface or component of an internal combustion engine, or an internal surface or component of a compression ignition engine.

10. The use of claim 8 or 9 wherein the lubricated surface is a lubricated surface of a motor vehicle.

11. Use of a lubricant composition of one of claims 1 to 7 in a vehicle having moving parts and containing a lubricant for lubricating the moving parts.

12. The use of claim 11, wherein the moving parts comprise a heavy duty diesel engine including exhaust gas recirculation and a lubricating system for the engine.

13. A method for improving the viscosity index of a lubricant composition comprising mixing with the lubricant composition from about 5 to about 30 percent by weight of an additive comprising a shear stable olefin copolymer derived from a copolymer having a number average molecular weight ranging from about 50,000 to about 250,000, wherein the shear stable olefin copolymer has a shear stability index of less than about 40, a polydispersity of not more than about 1.5, and a thickening efficiency of greater than about 1.8, and wherein the amount of additiv in the lubricant composition is based on a total weight of the lubricant composition.

14. The method of claim 13, wherein the lubricant composition comprises a multi-viscosity lubricating oil.

15. The method of claim 13, wherein the shear stable copolymer is defined as in one of claims 3 to 7.

16. A lubricant additive concentrate comprising a diluent or carrier oil and from about 5 to about 90 percent by weight of an additive comprising a shear stable olefin copolymer derived from a copolymer having a number average molecular weight ranging from about 50,000 to about 250,000, wherein the shear stable olefin copolymer has a shear stability index of less than about 40, a polydispersity of not more than about 1.5, and a thickening efficiency of greater than about 1.8.

17. The additive concentrate of claim 16, wherein the shear stable copolymer is as defined in one of claims 3 to 7.

18. The lubricant composition of claim 1 comprising a base oil and the additive concentrate of claim 16 or 17.

19. A method of lubricating moving parts comprising contacting the moving parts with a lubricant composition as defined in one of claims 1 to 7 or 19.

20. The method of claim 19 wherein the moving parts comprise one or more moving parts of a vehicle.

21. The method of claim 20 wherein the vehicle includes a diesel engine and wherein the moving parts include moving parts of the engine, or wherein the vehicle includes a marine vehicle having an engine, and wherein the moving parts include moving parts of the engine, or wherein the vehicle includes a spark ignition engine, and wherein the moving parts include moving parts of the engine

22. The method of claim 20, wherein the vehicle includes a drive train, and wherein the moving parts include moving parts of the drive train.

23. The method of claim 20, wherein the vehicle includes an internal combustion engine having a crankcase and wherein the lubricant composition comprises a crankcase oil present in the crankcase of the vehicle.

24. The method of claim 20, wherein the lubricant composition comprises a drive train lubricant present in an automotive drive train of the vehicle.
